# EUROPEAN PATENT SPECIFICATION

(11) **EP 3 040 459 B1**
(45) Date of publication and mention of the grant of the patent: **06.07.2022**
(21) Application number: 15199742.6
(22) Date of filing: 14.12.2015
(51) Int. Cl.: D04B 1/12

(54) **DOUBLE FLEECE KNIT FABRIC**
DOPPELVLIESSTRICKSTOFF
TRICOT MOLLETONNÉ DOUBLE

(30) Priority: 19.12.2014 JP 2014257111
(43) Date of publication of application: 06.07.2016
(73) Proprietor: Precision Fukuhara Works, Ltd., Kobe-shi Hyogo 651-2242 (JP)
(72) Inventor: TSUJIGO, Jun, Kobe-shi Hyogo 651-2242 (JP); ENISHI, Masaru, Kobe-shi Hyogo 651-2242 (JP)
(74) Representative: Rupprecht, Kay

(56) References cited:
- WO-A1-2009/136063
- US-A- 5 508 098

## Description

### BACKGROUND OF THE INVENTION

### 1. Field of the Invention

The present invention relates to a double fleece knit fabric produced on the knitting head of a circular knitting machine. In particular, the present invention relates to a knit fabric with an elaborate and decorative design having a Jacquard mesh pattern with concavity and convexity on the face side.

### 2. Description of Related Art

Generally, double fleece knit fabrics produced on the knitting head of a circular knitting machine are composed of inlay yarns that are held down by tie-in loops and further overlapped and intertwined by knit-in loops. Such fabrics are characterized in that tie-in loops composed of tie-in yarns appear on the face side of the knit fabrics but inlay yarns do not appear on the face side. Since such fabrics are knitted using three kinds of yarns consisting of inlay, tie-in, and knit-in yarns, they are called "3-end fleeces" or "3-thread fleeces" Exemplarily, knitted fabrics are known from prior art documents US 5,508,098 A and WO 2009/136063 A1.

Typical inlay patterns on the back side of such knit fabrics are 1×1 staggered, 2x1 twill, and 3x1 staggered, and some knitting machines are capable of making inlay yarns appear in a Jacquard style.

### Conventional Technique 1

FIG. 1 shows a 3x1 staggered double fleece knit fabric, and Table 1 shows a knitting notation of the same fabric.

In the table, code ∘ refers to a knit loop, • refers to a tuck loop of an inlay yarn, - refers to a welt of an inlay yarn, and W refers to a welt of a knit-in yarn. Code B refers to a block. For convenience, three successive courses consisting of an inlay yarn course, a tie-in yarn course and a knit-in yarn course are taken as one block. Code C refers to a course composed of successive loops arranged in the horizontal direction of the knit fabric. Although not given a code, successive loops arranged in the vertical direction of the knit fabric are referred to as a wale.

FIG. 8 shows a schematic view of a knit fabric cross-section according to Conventional Technique 1. All tie-in loops composed of a tie-in yarn and all knit-in loops composed of a knit-in yarn are knitted, and, thus, concavity and convexity do not appear on the face side and the back side of the knit fabric.

### Conventional Technique 2

Conventional Technique 2 described below is Example 1 (3x1 staggered double fleece (mesh) knit fabric) of JP 2010-24607A by the applicant of the present invention.

In FIG. 2 and Table 2, an inlay yarn (A1) of a first block is tucked in a first wale and welted in second to fourth wales, and repeats this sequence. A tie-in yarn (A2) of the first block is knitted in all wales, and repeats this sequence. A knit-in yarn (A3) of the first block is knitted in the first and second wales, welted in the third wale, and knitted in the fourth wale, and repeats this sequence.

An inlay yarn (A4) of a second block is welted in the first and second wales, tucked in the third wale, and welted in the fourth wale, and repeats this sequence. A tie-in yarn (A5) of the second block is knitted in all wales, and repeats this sequence. A knit-in yarn (A6) of the second block is knitted in the first and second wales, welted in the third wale, and knitted in the fourth wale, and repeats this sequence.

An inlay yarn (A7) of a third block is tucked in the first wale and welted in the second to fourth wales, and repeats this sequence. A tie-in yarn (A8) of the third block is knitted in all wales, and repeats this sequence. A knit-in yarn (A9) of the third block is welted in the first wale and knitted in the second to fourth wales, and repeats this sequence.

An inlay yarn (A10) of a fourth block is welted in the first and second wales, tucked in the third wale, and welted in the fourth wale, and repeats this sequence. A tie-in yarn (A11) of the fourth block is knitted in all wales, and repeats this sequence. A knit-in yarn (A12) of the fourth block is welted in the first wale and knitted in the second to fourth wales, and repeats this sequence.

In this manner, twelve courses make up a repeat of patterns.

FIG. 9 shows a schematic view of a knit fabric cross-section according to Conventional Technique 2. All tie-in loops composed of a tie-in yarn are knitted, and, thus, the face side of the knit fabric is flat and concavity and convexity do not appear thereon. Knit-in loops composed of a knit-in yarn have concavity at welted portions thereof but these portions are covered by an inlay yarn, and, thus, concavity and convexity do not clearly appear.

Although not described in detail in this specification, JP 2010-24607A further described the following three kinds of knit fabrics.
2x1 Twill double fleece (mesh) knit fabric (Example 2 of this document)
1×1 Staggered double fleece (mesh) knit fabric (Example 3 of this document)
3x1 Twill double fleece (mesh) knit fabric (Example 4 of this document)

The above knit fabrics, however, do not include a double fleece knit fabric that combines features of both Jacquard knitting of a mesh pattern with concavity and convexity on the face side and double fleece knitting on the back side, of a ground fabric composed of double-fleece-knitted tie-in loops and knit-in loops.

Generally, there has been a stereotype idea in which, in a double fleece knit fabric composed of three kinds of yarns consisting of inlay, tie-in, and knit-in yarns, all portions of the tie-in yarn arranged directly after the inlay yarn have to be knitted in order to fix tucked portions of the inlay yarn, but the present invention realizes a knit fabric in which only portions of the tie-in yarn arranged directly after tucked portions of the inlay yarn are knitted and the other portions of the tie-in yarn are either knitted or welted, thereby overturning this stereotype idea.

### SUMMARY OF THE INVENTION

In order to solve the above-described problem, the present invention is directed to a double fleece knit fabric according to claim 1.

It is preferable that, among an inlay yarn, a tie-in yarn, and a knit-in yarn that are successively arranged, the tie-in yarn in the same wale as the wale where the inlay yarn is welted is either knitted or welted, and the tie-in yarn in the same wale as the wale where the inlay yarn is tucked is knitted.

As described above, according to the knit fabric of the present invention, in double fleece knitting, a Jacquard pattern with concavity and convexity appears on the face side of a ground fabric composed of tie-in loops and knit-in loops. Accordingly, a knit fabric with an elaborate and decorative design is obtained that features good breathability and has features of Jacquard knitting of a mesh pattern with concavity and convexity on the face side of double fleece knitting for general clothing.

### BRIEF DESCRIPTION OF THE DRAWINGS

FIG. 1 shows a 3x1 staggered double fleece knit fabric of Conventional Technique 1 viewed from the back side.
FIG. 2 shows a 3x1 staggered double fleece (mesh) knit fabric of Conventional Technique 2 viewed from the back side.
FIG. 3 shows a 3x1 staggered-1 double fleece knit fabric of Example 1 of the present invention viewed from the back side.
FIG. 4 shows a 3x1 staggered-2 double fleece knit fabric of Example 2 of the present invention viewed from the back side.
FIG. 5 shows a 2x1 staggered-1 double fleece knit fabric of Example 3 of the present invention o viewed from the back side.
FIG. 6 shows a 2x1 staggered-2 double fleece knit fabric of Example 4 of the present invention viewed from the back side.
FIG. 7 shows a 2x1 staggered-3 double fleece knit fabric of Example 5 of the present invention viewed from the back side.
FIG. 8 shows a schematic view of a knit fabric cross-section according to Conventional Technique 1.
FIG. 9 shows a schematic view of a knit fabric cross-section according to Conventional Technique 2.
FIG. 10 shows a schematic view of a knit fabric cross-section according to Example 1 of the present invention.

### DETAILED DESCRIPTION OF THE INVENTION

Hereinafter, preferred embodiments of the present invention will be described with reference to the tables and drawings. Codes used in the tables are as described above.

The knit fabrics of the following examples can be produced using a known double fleece knitting machine and applying the settings of the present invention. Examples of such a double fleece knitting machine include MXC-RS3.2DF manufactured by Precision Fukuhara Works, Ltd. (Kobe, Japan). Cotton yarn 10/1 was used as the inlay yarns, cotton yarn 30/1 was used as the tie-in yarns, and polyester 56Dtex/24F was used as the knit-in yarns.

### Example 1

Next, FIG. 3 and Table 3 corresponding to Example 1 of the present invention will be described.

In FIG. 3 and Table 3, an inlay yarn (E1) of a first block is tucked in a first wale and welted in second to fourth wales, and repeats this sequence. A tie-in yarn (E2) of the first block is knitted in the first and second wales, welted in the third wale, and knitted in the fourth wale, and repeats this sequence. A knit-in yarn (E3) of the first block is knitted in all wales, and repeats this sequence.

An inlay yarn (E4) of a second block is welted in the first and second wales, tucked in the third wale, and welted in the fourth wale, and repeats this sequence. A tie-in yarn (E5) of the second block is welted in the first wale and knitted in the second to fourth wales, and repeats this sequence. A knit-in yarn (E6) of the second block is knitted in all wales, and repeats this sequence.

In this manner, six courses make up a repeat of patterns.

FIG. 10 shows a schematic view of a knit fabric cross-section according to Example 1 of the present invention. Tie-in loops composed of a tie-in yarn have concavity at welted portions thereof, and concavity and convexity clearly appear. Furthermore, if yarns having different colors are respectively used as the tie-in yarn and the knit-in yarn, Jacquard knitting is realized because the knit-in loops are seen through at the welted portions of the tie-in loops from the face side of the knit fabric. Furthermore, if a yarn that is thinner than the tie-in yarn is used as the knit-in yarn, a knit fabric with a mesh pattern can be produced. The same is applied to the following examples.

### Example 2

Next, FIG. 4 and Table 4 corresponding to Example 2 of the present invention will be described.

In FIG. 4 and Table 4, an inlay yarn (F1) of a first block is tucked in a first wale and welted in second to fourth wales, and repeats this sequence. A tie-in yarn (F2) of the first block is knitted in the first wale and welted in the second wale, and repeats this sequence. A knit-in yarn (F3) of the first block is knitted in all wales, and repeats this sequence.

An inlay yarn (F4) of a second block is welted in the first and second wales, tucked in the third wale, and welted in the fourth wale, and repeats this sequence. A tie-in yarn (F5) of the second block is knitted in the first wale and welted in the second wale, and repeats this sequence. A knit-in yarn (F6) of the second block is knitted in all wales, and repeats this sequence.

In this manner, six courses make up a repeat of patterns.

### Example 3

Next, FIG. 5 and Table 5 corresponding to Example 3 of the present invention will be described.

In FIG. 5 and Table 5, an inlay yarn (G1) of a first block is tucked in a first wale and welted in second and third wales, and repeats this sequence. A tie-in yarn (G2) of the first block is knitted in the first and second wales and welted in the third wale, and repeats this sequence. A knit-in yarn (G3) of the first block is knitted in all wales, and repeats this sequence.

An inlay yarn (G4) of a second block is welted in the first wale, tucked in the second wale, and welted in the third wale, and repeats this sequence. A tie-in yarn (G5) of the second block is knitted in the first and second wales and welted in the third wale, and repeats this sequence. A knit-in yarn (G6) of the second block is knitted in all wales, and repeats this sequence.

An inlay yarn (G7) of a third block is welted in the first and second wales and tucked in the third wale, and repeats this sequence. A tie-in yarn (G8) of the third block is knitted in the first wale, welted in the second wale, and knitted in the third wale, and repeats this sequence. A knit-in yarn (G9) of the third block is knitted in all wales, and repeats this sequence.

An inlay yarn (G10) of a fourth block is tucked in the first wale and welted in the second and third wales, and repeats this sequence. A tie-in yarn (G11) of the fourth block is knitted in the first wale, welted in the second wale, and knitted in the third wale, and repeats this sequence. A knit-in yarn (G12) of the fourth block is knitted in all wales, and repeats this sequence.

An inlay yarn (G13) of a fifth block is welted in the first wale, tucked in the second wale, and welted in the third wale, and repeats this sequence. A tie-in yarn (G14) of the fifth block is welted in the first wale and knitted in the second and third wales, and repeats this sequence. A knit-in yarn (G15) of the fifth block is knitted in all wales, and repeats this sequence.

An inlay yarn (G16) of a sixth block is welted in the first and second wales and tucked in the third wale, and repeats this sequence. A tie-in yarn (G17) of the sixth block is welted in the first wale and knitted in the second and third wales, and repeats this sequence. A knit-in yarn (G18) of the sixth block is knitted in all wales, and repeats this sequence.

In this manner, 18 courses make up a repeat of patterns.

### Example 4

Next, FIG. 6 and Table 6 corresponding to Example 4 of the present invention will be described.

In FIG. 6 and Table 6, an inlay yarn (H1) of a first block is tucked in a first wale and welted in second and third wales, and repeats this sequence. A tie-in yarn (H2) of the first block is knitted in the first and second wales and welted in the third wale, and repeats this sequence. A knit-in yarn (H3) of the first block is knitted in all wales, and repeats this sequence.

An inlay yarn (H4) of a second block is welted in the first wale, tucked in the second wale, and welted in the third wale, and repeats this sequence. A tie-in yarn (H5) of the second block is welted in the first wale and knitted in the second and third wales, and repeats this sequence. A knit-in yarn (H6) of the second block is knitted in all wales, and repeats this sequence.

An inlay yarn (H7) of a third block is welted in the first and second wales and tucked in the third wale, and repeats this sequence. A tie-in yarn (H8) of the third block is knitted in the first wale, welted in the second wale, and knitted in the third wale, and repeats this sequence. A knit-in yarn (H9) of the third block is knitted in all wales, and repeats this sequence.

In this manner, nine courses make up a repeat of patterns.

### Example 5

Next, FIG. 7 and Table 7 corresponding to Example 5 of the present invention will be described.

In FIG. 7 and Table 7, an inlay yarn (I1) of a first block is tucked in a first wale and welted in second and third wales, and repeats this sequence. A tie-in yarn (12) of the first block is knitted in the first and second wales and welted in the third wale, and repeats this sequence. A knit-in yarn (13) of the first block is knitted in all wales, and repeats this sequence.

An inlay yarn (14) of a second block is welted in the first wale, tucked in the second wale, and welted in the third wale, and repeats this sequence. A tie-in yarn (15) of the second block is knitted in the first and second wales and welted in the third wale, and repeats this sequence. A knit-in yarn (16) of the second block is knitted in all wales, and repeats this sequence.

An inlay yarn (17) of a third block is welted in the first and second wales and tucked in the third wale, and repeats this sequence. A tie-in yarn (18) of the third block is knitted in all wales, and repeats this sequence. A knit-in yarn (19) of the third block is knitted in all wales, and repeats this sequence.

In this manner, nine courses make up a repeat of patterns.

The present invention is not limited to the foregoing embodiments, and various modifications are possible within the scope of the claims. Also in these modifications other than the embodiments, a Jacquard pattern with concavity and convexity on the face side can be freely expressed in a double fleece knit fabric characterized in that, among an inlay yarn, a tie-in yarn, and a knit-in yarn that are successively arranged, the tie-in yarn in the same wale as the wale where the inlay yarn is welted is either knitted or welted, and the tie-in yarn in the same wale as the wale where the inlay yarn is tucked is knitted.

### List of Reference Numerals

- A1, A4, A7, A10: Inlay yarn of Conventional Technique 2
- A2, A5, A8, A11: Tie-in yarn of Conventional Technique 2
- A3, A6, A9, A12: Knit-in yarn of Conventional Technique 2
- E1, E4: Inlay yarn of Example 1 of the invention
- E2, E5: Tie-in yarn of Example 1 of the invention
- E3, E6: Knit-in yarn of Example 1 of the invention
- F1, F4: Inlay yarn of Example 2 of the invention
- F2, F5: Tie-in yarn of Example 2 of the invention
- F3, F6: Knit-in yarn of Example 2 of the invention
- G1, G4, G7, G10, G13, G16: Inlay yarn of Example 3 of the invention
- G2, G5, G8, G11, G14, G17: Tie-in yarn of Example 3 of the invention
- G3, G6, G9, G12, G15, G18: Knit-in yarn of Example 3 of the invention
- H1, H4, H7: Inlay yarn of Example 4 of the invention
- H2, H5, H8: Tie-in yarn of Example 4 of the invention
- H3, H6, H9: Knit-in yarn of Example 4 of the invention
- I1, 14, I7: Inlay yarn of Example 5 of the invention
- I2, I5, I8: Tie-in yarn of Example 5 of the invention
- I3, I6, I9: Knit-in yarn of Example 5 of the invention

## Claims

1. A double fleece knit fabric composed of three kinds of yarns consisting of inlay, tie-in, and knit-in yarns,
wherein the inlay yarn is held down by a tie-in loop on the face side and further overlapped and intertwined by a knit-in loop on the back side, **characterised in that**
the tie-in yarn is knitted and welted, and the knit-in yarn is all knitted.

2. The double fleece knit fabric according to claim 1,
wherein, among an inlay yarn, a tie-in yarn, and a knit-in yarn that are successively arranged, the tie-in yarn in the same wale as the wale where the inlay yarn is welted is either knitted or welted, and the tie-in yarn in the same wale as the wale where the inlay yarn is tucked is knitted.

3. The double fleece knit fabric according to claim 2,
wherein the pattern of the inlays is 2x1 welt/tuck.

4. The double fleece knit fabric according to claim 2,
wherein the pattern of the inlays is 3x1 welt/tuck.

5. A double fleece knit fabric according to claim 1 in which six courses make up a repeat of
patterns, wherein
- an inlay yarn of a first block is tucked in a first wale and welted in second to fourth wales, and repeats this sequence, a tie-in yarn of the first block is knitted in the first and second wales, welted in the third wale, and knitted in the fourth wale, and repeats this sequence, and a knit-in yarn of the first block is knitted in all wales, and repeats this sequence,
- after which an inlay yarn of a second block is welted in the first and second wales, tucked in the third wale, and welted in the fourth wale, and repeats this sequence, a tie-in yarn of the second block is welted in the first wale and knitted in the second to fourth wales, and repeats this sequence, and a knit-in yarn of the second block is knitted in all wales, and repeats this sequence.

6. A double fleece knit fabric according to claim 1 in which six courses make up a repeat of
patterns, wherein
- an inlay yarn of a first block is tucked in a first wale and welted in second to fourth wales, and repeats this sequence, a tie-in yarn of the first block is knitted in the first wale and welted in the second wale, and repeats this sequence, and a knit-in yarn of the first block is knitted in all wales, and repeats this sequence,
- after which an inlay yarn of a second block is welted in the first and second wales, tucked in the third wale, and welted in the fourth wale, and repeats this sequence, a tie-in yarn of the second block is knitted in the first wale and welted in the second wale, and repeats this sequence, and a knit-in yarn of the second block is knitted in all wales, and repeats this sequence.

7. A double fleece knit fabric according to claim 1 in which 18 courses make up a repeat of
patterns, wherein
- an inlay yarn of a first block is tucked in a first wale and welted in second and third wales, and repeats this sequence, a tie-in yarn of the first block is knitted in the first and second wales and welted in the third wale, and repeats this sequence, and a knit-in yarn of the first block is knitted in all wales, and repeats this sequence,
- after which an inlay yarn of a second block is welted in the first wale, tucked in the second wale, welted in the third wale, and repeats this sequence, a tie-in yarn of the second block is knitted in the first and second wales and welted in the third wale, and repeats this sequence, and a knit-in yarn of the second block is knitted in all wales, and repeats this sequence,
- after which an inlay yarn of a third block is welted in the first and second wales and tucked in the third wale, and repeats this sequence, a tie-in yarn of the third block is knitted in the first wale, welted in the second wale, and knitted in the third wale, and repeats this sequence, and a knit-in yarn of the third block is knitted in all wales, and repeats this sequence,
- after which an inlay yarn of a fourth block is tucked in the first wale and welted in the second and third wales, and repeats this sequence, a tie-in yarn of the fourth block is knitted in the first wale, welted in the second wale, and knitted in the third wale, and repeats this sequence, and a knit-in yarn of the fourth block is knitted in all wales, and repeats this sequence,
- after which an inlay yarn of a fifth block is welted in the first wale, tucked in the second wale, and welted in the third wale, and repeats this sequence, a tie-in yarn of the fifth block is welted in the first wale and knitted in the second and third wales, and repeats this sequence, and a knit-in yarn of the fifth block is knitted in all wales, and repeats this sequence,
- after which an inlay yarn of a sixth block is welted in the first and second wales and tucked in the third wale, and repeats this sequence, a tie-in yarn of the sixth block is welted in the first wale and knitted in the second and third wales, and repeats this sequence, and a knit-in yarn of the sixth block is knitted in all wales, and repeats this sequence.

8. A double fleece knit fabric according to claim 1 in which nine courses make up a repeat of
patterns, wherein
- an inlay yarn of a first block is tucked in a first wale and welted in second and third wales, and repeats this sequence, a tie-in yarn of the first block is knitted in the first and second wales and welted in the third wale, and repeats this sequence, and a knit-in yarn of the first block is knitted in all wales, and repeats this sequence,
- after which an inlay yarn of a second block is welted in the first wale, tucked in the second wale, and welted in the third wale, and repeats this sequence, a tie-in yarn of the second block is welted in the first wale and knitted in the second and third wales, and repeats this sequence, and a knit-in yarn of the second block is knitted in all wales, and repeats this sequence,
- after which an inlay yarn of a third block is welted in the first and second wales and tucked in the third wale, and repeats this sequence, a tie-in yarn of the third block is knitted in the first wale, welted in the second wale, and knitted in the third wale, and repeats this sequence, and a knit-in yarn of the third block is knitted in all wales, and repeats this sequence.

9. A double fleece knit fabric according to claim 1 in which nine courses make up a repeat of
patterns, wherein
- an inlay yarn of a first block is tucked in a first wale and welted in second and third wales, and repeats this sequence, a tie-in yarn of the first block is knitted in the first and second wales and welted in the third wale, and repeats this sequence, and a knit-in yarn of the first block is knitted in all wales, and repeats this sequence,
- after which an inlay yarn of a second block is welted in the first wale, tucked in the second wale, and welted in the third wale, and repeats this sequence, a tie-in yarn of the second block is knitted in the first and second wales and welted in the third wale, and repeats this sequence, and a knit-in yarn of the second block is knitted in all wales, and repeats this sequence,
- after which an inlay yarn of a third block is welted in the first and second wales and tucked in the third wale, and repeats this sequence, a tie-in yarn of the third block is knitted in all wales, and repeats this sequence, and a knit-in yarn of the third block is knitted in all wales, and repeats this sequence.

## Patentansprüche

1. Doppelvliesstrickstoff, zusammengesetzt aus drei Arten von Garnen, die aus Einlegegarn, Einbindegarn und Einstrickgarn bestehen,
wobei das Einlegegarn durch eine Einbindemasche auf der Stirnseite niedergehalten wird und außerdem durch eine Einstrickmasche auf der Rückseite überdeckt und verflochten wird, **dadurch gekennzeichnet, dass**
das Einbindegarn gestrickt und gesäumt wird, und das Einstrickgarn ganz gestrickt wird.

2. Doppelvliesstrickstoff nach Anspruch 1,
wobei unter einem Einlegegarn, einem Einbindegarn und einem Einstrickgarn, die aufeinanderfolgend angeordnet sind, das Einbindegarn im gleichen Maschenstäbchen wie das Maschenstäbchen, in dem das Einlegegarn gesäumt ist, entweder gestrickt oder gesäumt wird, und das Einbindegarn im gleichen Maschenstäbchen wie das Maschenstäbchen, in dem das Einlegegarn eingeschlagen ist, gestrickt wird.

3. Doppelvliesstrickstoff nach Anspruch 2, wobei das Muster der Einlagen 2x1 Einfassung/Abnäher ist.

4. Doppelvliesstrickstoff nach Anspruch 2, wobei das Muster der Einlagen 3x1 Einfassung/Abnäher ist.

5. Doppelvliesstrickstoff nach Anspruch 1, bei dem sechs Maschenreihen eine Wiederholung von Mustern ausmachen, wobei
- ein Einlegegarn eines ersten Blocks in einem ersten Maschenstäbchen eingeschlagen und im zweiten bis vierten Maschenstäbchen gesäumt ist, und diese Reihenfolge wiederholt, ein Einbindegarn des ersten Blocks in den ersten und zweiten Maschenstäbchen gestrickt, im dritten Maschenstäbchen gesäumt und im vierten Maschenstäbchen gestrickt ist, und diese Reihenfolge wiederholt, und ein Einstrickgarn des ersten Blocks in allen Maschenstäbchen gestrickt ist, und diese Reihenfolge wiederholt,
- nach welcher ein Einlegegarn eines zweiten Blocks im ersten und zweiten Maschenstäbchen gesäumt, im dritten Maschenstäbchen eingeschlagen und im vierten Maschenstäbchen gesäumt wird, und diese Reihenfolge wiederholt, ein Einbindegarn des zweiten Blocks im ersten Maschenstäbchen gesäumt und im zweiten bis vierten Maschenstäbchen gestrickt wird, und diese Reihenfolge wiederholt, und ein Einstrickgarn des zweiten Blocks in allen Maschenstäbchen gestrickt wird, und diese Reihenfolge wiederholt.

6. Doppelvliesstrickstoff nach Anspruch 1, bei dem sechs Maschenreihen eine Wiederholung von Mustern ausmachen, wobei
- ein Einlegegarn eines ersten Blocks in einem ersten Maschenstäbchen eingeschlagen und im zweiten bis vierten Maschenstäbchen gesäumt wird, und diese Reihenfolge wiederholt, ein Einbindegarn des ersten Blocks im ersten Maschenstäbchen gestrickt und im zweiten Maschenstäbchen gesäumt wird, und diese Reihenfolge wiederholt, und ein Einstrickgarn des ersten Blocks in allen Maschenstäbchen gestrickt wird, und diese Reihenfolge wiederholt,
- nach welcher ein Einlegegarn eines zweiten Blocks im ersten und zweiten Maschenstäbchen gesäumt, im dritten Maschenstäbchen eingeschlagen und im vierten Maschenstäbchen gesäumt wird, und diese Reihenfolge wiederholt, ein Einbindegarn des zweiten Blocks im ersten Maschenstäbchen gestrickt und im zweiten Maschenstäbchen gesäumt wird, und diese Reihenfolge wiederholt, und ein Einstrickgarn des zweiten Blocks in allen Maschenstäbchen gestrickt wird, und diese Reihenfolge wiederholt.

7. Doppelstrickvliesstrickstoff nach Anspruch 1, bei dem 18 Maschenreihen eine Wiederholung von Mustern ausmachen, wobei
- ein Einlegegarn eines ersten Blocks in einem ersten Maschenstäbchen eingeschlagen und im zweiten und dritten Maschenstäbchen gesäumt wird, und diese Reihenfolge wiederholt, ein Einbindegarn des ersten Blocks im ersten und zweiten Maschenstäbchen gestrickt und im dritten Maschenstäbchen gesäumt wird, und diese Reihenfolge wiederholt, und ein Einstrickgarn des ersten Blocks in allen Maschenstäbchen gestrickt wird, und diese Reihenfolge wiederholt,
- nach welcher ein Einlegegarn eines zweiten Blocks im ersten Maschenstäbchen gesäumt, im zweiten Maschenstäbchen eingeschlagen, im dritten Maschenstäbchen gesäumt wird, und diese Reihenfolge wiederholt, ein Einbindegarn des zweiten Blocks im ersten und zweiten Maschenstäbchen gestrickt und im dritten Maschenstäbchen gesäumt wird, und diese Reihenfolge wiederholt, und ein Einstrickgarn des zweiten Blocks in allen Maschenstäbchen gestrickt wird, und diese Reihenfolge wiederholt,
- nach welcher ein Einlegegarn eines dritten Blocks im ersten und zweiten Maschenstäbchen gesäumt und im dritten Maschenstäbchen eingeschlagen wird, und diese Reihenfolge wiederholt, ein Einbindegarn des dritten Blocks im ersten Maschenstäbchen gestrickt, im zweiten Maschenstäbchen gesäumt und im dritten Maschenstäbchen gestrickt wird, und diese Reihenfolge wiederholt, und ein Einstrickgarn des dritten Blocks in allen Maschenstäbchen gestrickt wird, und diese Reihenfolge wiederholt,
- nach welcher ein Einlegegarn eines vierten Blocks im ersten Maschenstäbchen eingeschlagen und im zweiten und dritten Maschenstäbchen gesäumt wird, und diese Reihenfolge wiederholt, ein Einbindegarn des vierten Blocks im ersten Maschenstäbchen gestrickt, im zweiten Maschenstäbchen gesäumt und im dritten Maschenstäbchen gestrickt wird, und diese Reihenfolge wiederholt, und ein Einstrickgarn des vierten Blocks in allen Maschenstäbchen gestrickt wird, und diese Reihenfolge wiederholt,
- nach welcher ein Einlegegarn eines fünften Blocks im ersten Maschenstäbchen gesäumt, im zweiten Maschenstäbchen eingeschlagen und im dritten Maschenstäbchen gesäumt wird, und diese Reihenfolge wiederholt, ein Einbindegarn des fünften Blocks im ersten Maschenstäbchen gesäumt und im zweiten und dritten Maschenstäbchen gestrickt wird, und diese Reihenfolge wiederholt, und ein Einstrickgarn des fünften Blocks in allen Maschenstäbchen gestrickt wird, und diese Reihenfolge wiederholt,
- nach welcher ein Einlegegarn eines sechsten Blocks im ersten und zweiten Maschenstäbchen gesäumt und im dritten Maschenstäbchen eingeschlagen wird, und diese Reihenfolge wiederholt, ein Einbindegarn des sechsten Blocks im ersten Maschenstäbchen gesäumt und im zweiten und dritten Maschenstäbchen gestrickt wird, und diese Reihenfolge wiederholt, und ein Einstrickgarn des sechsten Blocks in allen Maschenstäbchen gestrickt wird, und diese Reihenfolge wiederholt.

8. Doppelvliesstrickstoff nach Anspruch 1, bei dem neun Maschenreihen eine Wiederholung von Mustern ausmachen, wobei
- ein Einlegegarn eines ersten Blocks in einem ersten Maschenstäbchen eingeschlagen und im zweiten und dritten Maschenstäbchen gesäumt wird, und diese Reihenfolge wiederholt, ein Einbindegarn des ersten Blocks im ersten und zweiten Maschenstäbchen gestrickt und im dritten Maschenstäbchen gesäumt wird, und diese Reihenfolge wiederholt, und ein Einstrickgarn des ersten Blocks in allen Maschenstäbchen gestrickt wird, und diese Reihenfolge wiederholt,
- nach welcher ein Einlegegarn eines zweiten Blocks im ersten Maschenstäbchen gesäumt, im zweiten Maschenstäbchen eingeschlagen und im dritten Maschenstäbchen gesäumt wird, und diese Reihenfolge wiederholt, ein Einbindegarn des zweiten Blocks im ersten Maschenstäbchen gesäumt und im zweiten und dritten Maschenstäbchen gestrickt wird, und diese Reihenfolge wiederholt, und ein Einstrickgarn des zweiten Blocks in allen Maschenstäbchen gestrickt wird, und diese Reihenfolge wiederholt,
- nach welcher ein Einlegegarn eines dritten Blocks im ersten und zweiten Maschenstäbchen gesäumt und im dritten Maschenstäbchen eingeschlagen wird, und diese Reihenfolge wiederholt, ein Einbindegarn des dritten Blocks im ersten Maschenstäbchen gestrickt, im zweiten Maschenstäbchen gesäumt und im dritten Maschenstäbchen gestrickt wird, und diese Reihenfolge wiederholt, und ein Einstrickgarn des dritten Blocks in allen Maschenstäbchen gestrickt wird, und diese Reihenfolge wiederholt.

9. Doppelvliesstrickstoff nach Anspruch 1, bei dem neun Maschenreihen eine Wiederholung von Mustern ausmachen, wobei
- ein Einlagegaren eines ersten Blocks in einem ersten Maschenstäbchen eingeschlagen und im zweiten und dritten Maschenstäbchen gesäumt wird, und diese Reihenfolge wiederholt, ein Einbindegarn des ersten Blocks im ersten und zweiten Maschenstäbchen gestrickt und im dritten Maschenstäbchen gesäumt wird, und diese Reihenfolge wiederholt, und ein Einstrickgarn des ersten Blocks in allen Maschenstäben gestrickt wird, und diese Reihenfolge wiederholt,
- nach welcher ein Einlegegarn eines zweiten Blocks im ersten Maschenstäbchen gesäumt, im zweiten Maschenstäbchen eingeschlagen und im dritten Maschenstäbchen gesäumt wird, und diese Reihenfolge wiederholt, ein Einbindegarn des zweiten Blocks im ersten und zweiten Maschenstäbchen gestrickt und im dritten Maschenstäbchen gesäumt wird, und diese Reihenfolge wiederholt, und ein Einstrickgarn des zweiten Blocks in allen Maschenstäbchen gestrickt wird, und diese Reihenfolge wiederholt,
- nach welcher ein Einlegegarn eines dritten Blocks im ersten und zweiten Maschenstäbchen gesäumt und im dritten Maschenstäbchen eingeschlagen wird, und diese Reihenfolge wiederholt, ein Einbindegarn des dritten Blocks in allen Maschenstäbchen gestrickt wird, und diese Reihenfolge wiederholt, und ein Einstrickgarn des dritten Blocks in allen Maschenstäbchen gestrickt wird, und diese Reihenfolge widerholt.

## Revendications

1. Tricot molletonné double composé de trois types de fils, à savoir des fils de trame, des fils de piquetage et des fils de tricotage,
dans lequel le fil de trame est maintenu vers le bas par une boucle de piquetage sur la face avant et est en outre recouvert et entrelacé par une boucle de tricotage sur la face arrière,
**caractérisé en ce que** le fil de piquetage est tricoté et bordé, et le fil de tricotage est entièrement tricoté.

2. Tricot molletonné double selon la revendication 1,
dans lequel, parmi un fil de trame, un fil de piquetage et un fil de tricotage qui sont disposés successivement, le fil de piquetage dans le même rebord que le rebord où le fil de trame est bordé, est soit tricoté soit bordé, et le fil de piquetage dans le même rebord que le rebord où le fil de trame est plissé est tricoté.

3. Tricoté molletonné double selon la revendication 2,
dans lequel le motif des trames est de 2 × 1 bord/pli.

4. Tricot molletonné double selon la revendication 2,
dans lequel le motif des trames est de 3 × 1 bord/pli.

5. Tricot molletonné double selon la revendication 1,
dans lequel six courses constituent une répétition des motifs,
et
- un fil de trame d'un premier bloc est plissé dans un premier rebord et bordé dans les deuxième à quatrième rebords, et on répète cette séquence, un fil de piquetage du premier bloc est tricoté dans les premier et deuxième rebords, bordé dans le troisième rebord, et tricoté dans le quatrième rebord, et on répète cette séquence, et un fil de tricotage du premier bloc est tricoté dans tous les rebords, et on répète cette séquence,
- après quoi un fil de trame d'un deuxième bloc est bordé dans les premier et deuxième rebords, plissé dans le troisième rebord et bordé dans le quatrième rebord, et on répète cette séquence, un fil de piquetage du deuxième bloc est bordé dans le premier rebord et tricoté dans les deuxième à quatrième rebords, et on répète cette séquence, et un fil de tricotage du deuxième bloc est tricoté dans tous les rebords, et on répète cette séquence.

6. Tricot molletonné double selon la revendication 1,
dans lequel six courses constituent une répétition des motifs,
et
- un fil de trame d'un premier bloc est plissé dans un premier rebord et bordé dans les deuxième à quatrième rebords, et on répète cette séquence, un fil de piquetage du premier bloc est tricoté dans le premier rebord et bordé dans le deuxième rebord, et on répète cette séquence, et un fil de tricotage du premier bloc est tricoté dans tous les rebords, et on répète cette séquence,
- après quoi un fil de trame d'un deuxième bloc est bordé dans les premier et deuxième rebords, plissé dans le troisième rebord et bordé dans le quatrième rebord, et on répète cette séquence, un fil de piquetage du deuxième bloc est tricoté dans le premier rebord et bordé dans le deuxième rebord, et on répète cette séquence, et un fil de tricotage du deuxième bloc est tricoté dans tous les rebords, et on répète cette séquence.

7. Tricot molletonné double selon la revendication 1,
dans lequel 18 courses constituent une répétition des motifs,
et
- un fil de trame d'un premier bloc est plissé dans un premier rebord et bordé dans les deuxième et troisième rebords, et on répète cette séquence, un fil de piquetage du premier bloc est tricoté dans les premier et deuxième rebords et bordé dans le troisième rebord, et on répète cette séquence, et un fil de tricotage du premier bloc est tricoté dans tous les rebords, et on répète cette séquence,
- après quoi un fil de trame d'un deuxième bloc est bordé dans le premier rebord, plissé dans le deuxième rebord, bordé dans le troisième rebord, et on répète cette séquence, un fil de piquetage du deuxième bloc est tricoté dans les premier et deuxième rebords et bordé dans le troisième rebord, et on répète cette séquence, et un fil de tricotage du deuxième bloc est tricoté dans tous les rebords, et on répète cette séquence,
- après quoi un fil de trame d'un troisième bloc est bordé dans les premier et deuxième rebords et plissé dans le troisième rebord, et on répète cette séquence, un fil de piquetage du troisième bloc est tricoté dans le premier rebord, bordé dans le deuxième rebord et tricoté dans le troisième rebord, et on répète cette séquence, et un fil de tricotage du troisième bloc est tricoté dans tous les rebords, et on répète cette séquence,
- après quoi un fil de trame d'un quatrième bloc est plissé dans le premier rebord et bordé dans les deuxième et troisième rebords, et on répète cette séquence, un fil de piquetage du quatrième bloc est tricoté dans le premier rebord, bordé dans le deuxième rebord et tricoté dans le troisième rebord, et on répète cette séquence, et un fil de tricotage du quatrième bloc est tricoté dans tous les rebords, et on répète cette séquence,
- après quoi un fil de trame d'un cinquième bloc est bordé dans le premier rebord, plissé dans le deuxième rebord et bordé dans le troisième rebord, et on répète cette séquence, un fil de piquetage du cinquième bloc est bordé dans le premier rebord et tricoté dans les deuxième et troisième rebords, et on répète cette séquence, et un fil de tricotage du cinquième bloc est tricoté dans tous les rebords, et on répète cette séquence,
- après quoi un fil de trame d'un sixième bloc est bordé dans les premier et deuxième rebords et plissé dans le troisième rebord, et on répète cette séquence, un fil de piquetage du sixième bloc est bordé dans le premier rebord et tricoté dans les deuxième et troisième rebords, et on répète cette séquence, et un fil de tricotage du sixième bloc est tricoté dans tous les rebords, et on répète cette séquence.

8. Tricot molletonné double selon la revendication 1,
dans lequel neuf courses constituent une répétition des motifs,
et
- un fil de trame d'un premier bloc est plissé dans un premier rebord et bordé dans des deuxième et troisième rebords, et on répète cette séquence, un fil de piquetage du premier bloc est tricoté dans les premier et deuxième rebords et bordé dans le troisième rebord, et on répète cette séquence, et un fil de tricotage du premier bloc est tricoté dans tous les rebords, et on répète cette séquence,
- après quoi un fil de trame d'un deuxième bloc est bordé dans le premier rebord, plissé dans le deuxième rebord et bordé dans le troisième rebord, et on répète cette séquence, un fil de piquetage du deuxième bloc est bordé dans le premier rebord et tricoté dans les deuxième et troisième rebords, et on répète cette séquence, et un fil de tricotage du deuxième bloc est tricoté dans tous les rebords, et on répète cette séquence,
- après quoi, un fil de trame d'un troisième bloc est bordé dans les premier et deuxième rebords et plissé dans le troisième rebord, et on répète cette séquence, un fil de piquetage du troisième bloc est tricoté dans le premier rebord, bordé dans le deuxième rebord et tricoté dans le troisième rebord, et on répète cette séquence, et un fil de tricotage du troisième bloc est tricoté dans tous les rebords, et on répète cette séquence.

9. Tricot molletonné double selon la revendication 1,
dans lequel neuf courses constituent une répétition des motifs,
et
- un fil de trame d'un premier bloc est plissé dans un premier rebord et bordé dans les deuxième et troisième rebords, et on répète cette séquence, un fil de piquetage du premier bloc est tricoté dans les premier et deuxième rebords et bordé dans le troisième rebord, et on répète cette séquence, et un fil de tricotage du premier bloc est tricoté dans tous les rebords, et on répète cette séquence,
- après quoi un fil de trame d'un deuxième bloc est bordé dans le premier rebord, plissé dans le deuxième rebord et bordé dans le troisième rebord, et on répète cette séquence, un fil de piquetage du deuxième bloc est tricoté dans les premier et deuxième rebords et bordé dans le troisième rebord, et on répète cette séquence, et un fil de tricotage du deuxième bloc est tricoté dans tous les rebords, et on répète cette séquence,
- après quoi un fil de trame d'un troisième bloc est bordé dans les premier et deuxième rebords et plissé dans le troisième rebord, et on répète cette séquence, un fil de piquetage du troisième bloc est tricoté dans tous les rebords, et on répète cette séquence, et un fil de tricotage du troisième bloc est tricoté dans tous les rebords, et on répète cette séquence.
